

Aug. 21, 1928.

R. FRITSCHE

1,681,849

METHOD OF PREPARING RUST RESISTING IRON AND STEEL PRINTING PLATES

Filed April 7, 1927



Fig. 1.



Fig. 2.



Fig. 3.



Fig. 4.

Fig. 5.



Fig. 6.



Fig. 7.

WITNESSES  
George Maylor  
A. L. Ritchie

INVENTOR  
*Rudolf Fritsche*  
BY  
*Munn & Co.*  
ATTORNEY

Patented Aug. 21, 1928.

1,681,849

# UNITED STATES PATENT OFFICE.

RUDOLF FRITSCH, OF NEW YORK, N. Y.

## METHOD OF PREPARING RUST-RESISTING IRON AND STEEL PRINTING PLATES.

Application filed April 7, 1927. Serial No. 181,774.

This invention relates to producing lithographic plates using either the photographic method, the drawing or transfer method, and has for an object to provide improved steps 5 for producing a superior plate through the use of rust resisting iron, steel or similar metal.

Another object is to provide improved steps in the method of using rust resisting iron alloy which will not corrode appreciably the 10 water or many chemicals.

A further object of the invention is to provide an improved method and also finished plates for lithographing, wherein the improved steps include preparing a rust resisting iron and steel plate so as to readily receive the photographic coating or to readily receive and hold in place a transfer or a fatty hand drawing.

20 In the accompanying drawing—

Figure 1 is a plan view of a substantially rust-proof plate showing the formation of the plate greatly exaggerated, after the same has been washed by an alkaline solution.

25 Figure 2 is a sectional view through Figure 1, approximately on line 2—2.

Figure 3 is a view similar to Figure 2 but showing a sensitive photographic coating applied and ready to receive the photographic 30 impression.

Figure 4 is a view similar to Figure 2 but showing a modified form of plate produced by washing the plate with a different solution than that shown in Figure 2.

35 Figure 5 is a view similar to Figure 4 but showing a hand drawing and transfer applied.

Figure 6 is a view similar to Figure 5, but showing the plate with a protecting coating 40 of any well known kind, as for instance, a gum arabic solution.

Figure 7 is a perspective view of the structure shown in Figure 6, with half of the gum arabic solution removed.

45 Referring to the accompanying drawing by numerals, 1 indicates a metal plate, which may be a suitable form of rust resisting iron or steel, such as chrome iron alloy, silicon iron alloy and molybdenum iron alloy. After the 50 plate 1 has been secured, the same is washed with a solution for removing all grease and dirt so as to make the plate clean. A desired solution is ten per cent alkaline solution of a sodium (carbonate of soda) or potassium salt (carbonate of potash). A ten per cent solution is preferable as it secures the desired re-

sults in a minimum time without injury. A weaker solution could be used if desired, but would take a longer time to secure the desired result and even a stronger solution might be 60 used which would take less time but care would be necessary to prevent an injury to the plate.

The plate 1 is preferably grained in the usual manner and then washed with this solution. In washing the plate, the grease and dirt will be removed and also certain other particles, whereby slight indentations or pores 2 are formed. In the drawing, these indentations and also the grain, have been 70 greatly exaggerated as in a full size plate these indentations are so small that to the ordinary touch, the surface of a plate would feel smooth. After the plate 1 has been treated until it appears as shown in Figure 2, a sensitive coating 3 is applied thereto, said coating being any desired photographic coating now commonly used. After this coating has been applied, the plate is ready to be used in the usual manner in photolithographing. It 75 is to be understood that the picture is photographed directly on the solution 3 and then the solution is subjected to a developing or washing operation in a well known manner, after which, the plate is used in printing in a 80 well known manner.

During the printing operation as heretofore carried out with zinc and aluminum plates, there was considerable wearing away 85 of the plates caused by the water commonly used in printing and the chemicals in the printing solution. This wearing away of the zinc plates was really a slow etching which caused the lines of the work on the plate to become weaker so that the plate, after a certain usage, would make a poor reproduction 90 so that a new plate was necessary if a large number of copies were to be printed.

In printing with the plate 1 as shown in Figure 3, the water and chemicals used in the printing ink, will not affect plate 1 and, consequently, a very clear print is made and also a large number of prints may be made from the same plate.

In Figures 4 to 7 inclusive, a modified form 105 of the invention is shown, wherein the plate 1' is identical with the plate 1 except that the same has been washed with a different solution to produce the depressions or pores 2'. These parts have been greatly exaggerated, as a full size plate would be 110 comparatively smooth to the ordinary touch. In

producing plate 1', the same is made sensitive to fatty drawings or transfer impressions and this is done by using a mixture of hydrochloric acid and nitric acid. A desirable solution of these two acids is five to twenty-five per cent solution of a mixture of three parts hydrochloric acid and one part nitric acid. If desired, instead of this solution, a ten percent solution of hydrofluoric acid could be used. A stronger solution could be used of this kind up to a concentrated acid by reducing the time of treatment. Sometimes it is of advantage to use these two different solutions in succession and then wash and dry the plate. These treatments result in a plate as shown in Figure 4 which has a grained surface produced in the usual manner of graining and a porous surface to a certain limit, which causes the surface to be sensitive to fatty drawings or transfer impressions. The transfer impression may be placed in position in the usual manner as shown in Figure 5 so that the coating 3 will adhere firmly to the plate 1' and the supporting paper or other material 4 may be stripped off. The coating 5 is placed on the prepared surface by a pen or other instrument in the usual manner and may be a solid coating as shown in the drawing or may be in outline or partly in outline and partly solid. After the coatings 3 and 5 have been placed in position, the surface of the plate is then subjected to a coating of a gum arabic solution which will cover the entire surface of plate 1' except where the coatings 3 and 5 are positioned. This gum arabic coating 6 as shown in Figures 6 and 7, causes the entire surface to be a smooth even surface. When the inking roller is passed over the plate in the usual manner, ink will adhere to the coatings 3 and 5 so that a desired print may be secured. After the plate has been prepared as shown in Figures 6 and 7, it is in condition for printing in the usual press and in the usual manner. The only difference in printing, is that the plate is not injured by the water or chemicals in the printing ink and, consequently, many prints may be secured from the same plate and all of the prints will show a clear impression.

What I claim is:

1. A lithographic plate, comprising a chrome steel body formed with graining on one surface, with said grained surface having a porous formation. 55
2. The method of preparing a photolithographic plate, comprising the provision of a chrome steel plate, graining said plate, washing the plate with a solution of carbonate of potash until all grease and free dirt are removed, washing said plate with water until the alkaline solution has been all removed, drying said plate, and finally coating the plate with a photographic coating. 60
3. The method of producing a lithographic plate, comprising the production of a chrome steel plate, graining said plate, washing said plate with a 10% solution of carbonate of potash until the surface is somewhat porous, washing said plate with water until the solution has been all removed, and finally drying the plate. 65
4. The method of preparing lithographic plates, consisting in washing a rust-proof chrome steel plate to make the same sensitive to fatty drawings and transfer impressions, the washing being performed by a five to twenty-five per cent solution of a mixture of three parts hydrochloric acid and one part nitric acid, washing said solution off said plate by water, and finally drying the plate. 75
5. The method of forming a lithographic plate, consisting in providing a rust-proof chrome steel plate, washing one surface of the plate with a ten per cent solution of hydrofluoric acid, washing said acid off said plate with water, and finally drying the plate. 85
6. The method of forming a lithographic plate, consisting in providing a rust-proof chrome steel plate, making the surface of said plate sensitive to fatty drawings or transfer impressions by washing said surface with first a five to twenty-five per cent solution of mixture of three parts hydrochloric acid and one part nitric acid, and then washing the surface with a ten per cent solution of hydrofluoric acid, washing the various acids from the plate by the use of water, and finally drying the plate. 90
- 

RUDOLF FRITSCHE.